

## UNITED STATES PATENT OFFICE

2,221,641

## BLACK NICKEL FINISH

Burton Bower Knapp, Westfield, N. J., assignor to  
The International Nickel Company, Inc., New  
York, N. Y., a corporation of Delaware

No Drawing. Application November 13, 1939,  
Serial No. 304,142

23 Claims. (Cl. 148—6)

The present invention relates to chemically produced colored surfaces on articles having a nickel surface, to a bath suitable for the aforesaid purpose and to the products thereof.

5 It is recognized by those skilled in the art that the coloring of metals is an art. Accordingly it has not been possible in the past to lay down any set rules for obtaining various colors on metals. Fine craftsmanship and skill is required 10 of the operator to produce color effects. Special technique is involved in coloring and can only come from actual experience.

The composition of the metal will affect greatly the color to be obtained. Non-ferrous alloys 15 high in copper will take on different hues than those low in copper. Copper and alloys rich in copper can be more easily treated than alloys low in copper. It is necessary in some cases in order to obtain a particular shade to copper plate 20 the article before coloring. (Platers' Guidebook, 1938.)

In the 1939 edition of Platers' Guidebook, G. B. Hogaboom, Jr. and T. H. Chamberlain also indicate other factors which have heretofore only 25 been determined by experience. Thus on page 46 these authorities state that "Solution formulas may be varied and adjusted to suit particular conditions that will produce desired shades of color. Time of immersion and temperature are 30 other variables that are important and usually arrived at by experience. Many beautiful color effects are obtained in a great many instances by varying the procedure and sequence of operations." From the foregoing it will be appreciated 35 that the coloring of metals has not reached that stage of development at which generalizations might be made or prophecies given disclosing the manner in which certain color effects on particular metals may be obtained.

40 In both the 1938 edition and the 1939 edition of Platers' Guidebook, the composition of solutions and the conditions under which the coloring of silver, copper, brass, iron and steel is possible are given. Other solutions for the treatment 45 of non-ferrous metals are described in various U. S. Patents such as U. S. Patent Nos. 1,967,715, 2,001,753 and 2,012,697. For example, U. S. Patent No. 1,967,715 describes a solution suitable for depositing a corrosion resistant coating on a zinc base alloy and having the whitish appearance of the original uncoated alloy. A method for coating surfaces of copper by the action of organic acids is described in U. S. Patent No. 2,001,753. The use of acids including 50 oxalic and benzene-sulfonic acids for the coating

of non-ferrous metals such as lead, tin and cadmium is disclosed by Tanner and Lodeesen in U. S. Patent No. 2,012,697. The rust-proofing of iron and steel articles is described in U. S. Patent No. 2,105,672. None of the foregoing information provides the solution to the problem of providing articles in which the major constituent of the surface is nickel with an adherent black or colored coating. Nor am I aware that anyone has provided the art with a simplified, 5 accurately controlled process for providing articles having a surface constituted largely of nickel with a black or gray decorative and ornamental coating on an industrial scale by simple immersion capable of being employed by comparatively inexperienced operators. 10

It is an object of the present invention to provide a process for coloring or blackening nickel surfaces.

It is another object of the present invention to 20 provide a bath for coating nickel articles with an adherent black or colored ornamental and decorative film and having a bath efficiency indicator included therein.

The present invention also contemplates providing the art with nickel articles having a grayish to blackish surface, or having coatings of such thinness as to display interference phenomena.

Other objects and advantages will become apparent from the following description.

Broadly stated, the present invention provides a bath and process which even in inexperienced hands provides decorative surfaces on nickel articles. Operators lacking the experience in metal 35 coloring stressed by Hogaboom may produce highly ornamental coatings on articles having a nickel surface by taking advantage of the principles of the present invention.

The novel bath provided by the present invention permits the application of reduction and oxidation reactions to the production of the decorative black coatings on articles constituted of nickel. It is my opinion at this time that upon subjecting a nickel article to the action of the bath prepared in accordance with the principles of the present invention, a reducing condition is produced in the vicinity of, or at, and close to the surface of the article through the solution 50 of a small amount of nickel from the surface of the article. This reducing condition causes the formation of a black deposit on the surface of the article. Simultaneously, it is believed, an oxidation reaction takes place which may be said 55

to act as a scavenger and remove inhibiting reaction products.

I have found that suitable oxidizing agents for the purpose of the present invention are those oxidizing agents which at unit activity have an oxidation-reduction potential more negative than about -1.75 volts. During my investigation of the conditions under which articles having a nickel surface could be provided with black or colored films, the action of a number of oxidizing agents was investigated. I found that dichromates, chlorates, and permanganates gave unsatisfactory results when used in conjunction with the other components of my bath. On the other hand, hydrogen peroxide and persulfate gave satisfactory results. As those skilled in the art know, the oxidation-reduction potentials of these oxidizing agents are as follows:

|    |                   |       |
|----|-------------------|-------|
| 20 | Dichromate        | -1.36 |
|    | Chlorate          | -1.45 |
|    | Permanganate      | -1.67 |
|    | Hydrogen peroxide | -1.77 |
|    | Persulfate        | -2.05 |

25 Thus, it would appear that oxidizing agents having an oxidation-reduction potential less negative than about -1.75 do not give satisfactory results when used in accordance with the principles of the present invention.

30 In addition to materials capable of producing the foregoing reactions, I have found it preferable to include among the constituents of the bath a bath efficiency indicator. By means of this indicator it is possible to tell at a glance whether the 35 bath will produce the desired coatings or not when used in accordance with the principles of the present invention.

In order that those skilled in the art may have a better understanding of the principles of the 40 present invention, the following description is provided for illustrative purposes. I have found that a bath having an acidity of about pH 1 to pH 2 is necessary for the production of decorative or utilitarian coatings of articles consisting 45 of nickel or surfaced with nickel. In addition it is advantageous to include in the bath material capable of oxidizing at least one product of the reaction. I have found that in a bath such as described more fully hereinafter, both functions 50 can best be fulfilled by ammonium persulfate or hydrogen peroxide. When the latter is used, the pH changes less with use than where the persulfate is employed. To provide a source of sulfur ions, I have found the use of ammonium thio- 55 cyanate preferable. It is advantageous to stabilize a bath containing ammonium persulfate by the addition of a sulfate such as sodium sulfate. However, baths containing only ammonium persulfate or hydrogen peroxide and ammonium thio-cyanate have given satisfactory 60 results.

Other sulfur containing compounds may be substituted as a source of sulfur containing ions for the thio-cyanate. Among the class of sulfur 65 compounds suitable for this purpose are included sulfites, and thio-sulfates soluble in the bath and especially the alkaline salts thereof. A particular advantage accrues from the use of ammonium thio-cyanate in that by the use of a ferric salt, for 70 example, the sulfate, a visual indicator of the state of the bath is provided. Thus, in a bath containing both thio-cyanate and a ferric salt, the presence of thio-cyanate is clearly indicated by the red color. When the thio-cyanate is in 75 such low concentration as to render the bath

ineffective, the red color practically disappears. In the presence of a sulfate such as sodium sulfate, the persulfate is stable practically indefinitely, when the bath is idle, although it is consumed during use. However, the thio-cyanate 5 or other source of sulfur ions must be added from time to time as the concentration thereof falls below practical values. When a solution containing persulfate, thio-cyanate, alkali sulfate and a ferric salt is a deep red color, deep black 10 finishes may be produced on nickel by a five minute immersion therein at room temperature. As the film forms, a series of colors is produced by interference effect—those of the second order being particularly attractive. When these interference colors rather than gray or black are desired, it is best to use a bath containing low concentrations of thio-cyanate and/or ammonium persulfate or hydrogen peroxide, as such a bath 15 develops the film at a moderate rate, which 20 makes it easy to control the final color.

The simplest bath containing thio-cyanate and persulfate which has given satisfactory results is a 20% solution of ammonium persulfate containing 0.5% ammonium thio-cyanate. However, I 25 prefer to use a bath containing about 50 to about 200 grams ammonium persulfate per liter, about 25 to about 100 grams of sodium sulfate per liter, and about 1 to about 10 grams of ferric sulfate per liter. To the foregoing, ammonium thio- 30 cyanate is added from time to time in such amounts as to maintain the red color of the bath.

A bath which I have found to give very satisfactory black finishes in about 5 minutes has the following composition:

|                     |            |
|---------------------|------------|
| Ammonium persulfate | 200 gr/L * |
| Sodium sulfate      | 100 gr/L   |
| Ferric sulfate      | 10 gr/L    |

\*gr/L=grams per liter.

To the foregoing bath ammonium thio-cyanate is added from time to time in amounts sufficient to maintain a deep red color.

I have found that a bath for producing black 45 or colored finishes on nickel surfaces employing hydrogen peroxide as the oxidizing agent has several advantages over a persulfate bath. First, it simplifies the bath by reducing the number 50 of components therein, second, the pH of the bath may be more readily controlled. In this connection, it is of interest to note that while the persulfate bath tends to become more acidic during use, the hydrogen peroxide bath becomes more alkaline with use. Accordingly, I maintain 55 the pH of the peroxide bath substantially constant at about 1.2 by the addition of small amounts of sulfuric acid or by the use of a buffer, such as monochloracetic acid, orthophosphoric acid or the like in suitable amounts, for example, 60 about 10 grams per liter.

A bath having the following composition has given satisfactory results:

|                         |          |
|-------------------------|----------|
| Potassium sulfocyanate  | 0.5 gr/L |
| Sulfuric acid           | 5 gr/L   |
| Hydrogen peroxide (30%) | 25 cc pl |
| pH                      | 1.2      |

However, baths containing about 10 cc. to about 70 25 cc. per liter of 30% hydrogen peroxide and sufficient mineral acid to provide a pH of about 1 to about 2 and containing potassium-thio-cyanate or ammonium or alkali metal salts of the following sulfur containing acid, to wit: sulfuric and thio-sulfuric to be effective in pro- 75

ducing black or colored finishes on nickel surfaces have been found satisfactory.

While the foregoing baths may be used at about 15° to 20° C., higher bath temperatures 5 may be employed or the article to be treated may be warmed. At higher bath temperatures shorter periods of treatment suffice. However, the lower temperature is to be preferred, since there is decomposition of the bath at high temperatures. 10 By means of these baths and the process of the present invention, the careful control of conditions and the practically continual additions of salts required by the electrolytic processes for producing black nickel are eliminated and a 15 simpler and more reproducible method provided.

The process of the present invention is particularly applicable to the coloring of images on nickel strip or sheet. For this purpose the metal is coated with a light sensitive resist, printed, developed and etched. The etched image can then be colored black by means of any of the baths described hereinbefore. By this means a picture with good contrast and detail is obtained. Thus records can be made on time resistant nickel 20 film which last indefinitely. The method of the present invention can likewise be employed for the production of colors other than black for architectural uses. In the formation of the film on nickel a series of interference colors is formed 25 before the film acquires sufficient thickness to be jet black.

Although the present invention has been described in conjunction with certain preferred embodiments, it is to be understood that variations and modifications thereof may be made as those skilled in the art will readily understand. Such variations and modifications are to be considered within the purview of the present specification and the scope of the appended claims. 30 Thus, among the alkaline salts which may be employed as sources of sulfur are included ammonium and alkali metal salts of the thio-cyanates, sulfites and thio-sulfates. Furthermore, the expression, "nickel articles" as used herein 35 includes articles having a surface possessing a nickel content of at least about 95%.

I claim:

1. A process for producing decorative, ornamental and utilitarian finishes on nickel and 50 nickel surfaced articles which comprises immersing said articles in a bath having a pH of about 1 to about 2 and containing an oxidizing agent having at unit activity an oxidation-reduction potential more negative than about -1.75 55 volts and ammonium thio-cyanate in effective amounts and subjecting said articles to the action of said bath at a temperature of about 15° C. and higher for a period of time up to about 5 minutes.

2. A process for producing decorative, ornamental and utilitarian finishes on nickel and 60 nickel surfaced articles which comprises subjecting said articles to the action of a bath having a pH of about 1 to about 2 containing an oxidizing agent having at unit activity an oxidation-reduction potential more negative than about -1.75 volts and a reducible sulfur compound selected from the group consisting of thio-cyanates, sulfites, and thio-sulfates in effective amounts for a period of time at a temperature of about 15° C. and higher. 65

3. A process for producing decorative, ornamental and utilitarian finishes on nickel surfaced articles which comprises subjecting said articles 70 to the action of a bath containing about 50

to about 200 grams of ammonium persulfate and about 5 grams of ammonium thio-cyanate per liter at a temperature of at least 15° C. for a period of time not greater than about 5 minutes.

4. A process for producing decorative, ornamental and utilitarian finishes on nickel surfaced articles which comprises establishing a bath containing about 50 to about 200 grams of ammonium persulfate, about 25 to about 100 grams of sodium sulfate and about 1 to about 10 10 grams of ferric sulfate per liter and at least sufficient ammonium thio-cyanate to produce a red color in said bath, immersing nickel surfaced articles in said bath, maintaining said bath at a temperature of about 15° C. to about 20° C., 15 subjecting said nickel surfaced articles to the action of said bath for a period of time up to about 5 minutes, and adding ammonium thio-cyanate at intervals and in quantities sufficient to maintain the red color of said bath. 20

5. A process for producing decorative, ornamental, and utilitarian finishes on nickel surfaced articles which comprises establishing a bath containing about 50 grams to about 200 grams of ammonium persulfate, and an effective amount 25 of reducible sulfur compound selected from the group consisting of sulfates, thio-sulfates and thio-cyanates, and an ammonium persulfate stabilizing agent in effective amount, heating said bath to at least 15° C. and subjecting nickel 30 surfaced articles to the action of said bath for a period of time dependent upon the temperature thereof.

6. A process for producing decorative, ornamental and utilitarian finishes on nickel surfaced articles which comprises establishing a bath containing about 200 grams of ammonium persulfate, about 100 grams of sodium sulfate and about 10 grams of ferric sulfate per liter, adding at least sufficient ammonium thio-cyanate 40 to said bath to produce a red color therein and subjecting said nickel surfaced articles to the action of said red colored bath for a period of time up to about 5 minutes at a temperature of about 15° C. to about 20° C. 45

7. A bath suitable for producing decorative, ornamental or utilitarian finishes on nickel and nickel surfaced articles which comprises an oxidizing agent having at unit activity an oxidation-reduction potential of at least -1.75 volts in 50 effective amounts and a reducible sulfur compound in effective amounts, said bath having a pH of about 1 to about 2.

8. A bath suitable for producing decorative, ornamental or utilitarian finishes on nickel and 55 nickel surfaced articles and containing an oxidizing agent selected from the group consisting of hydrogen peroxide and ammonium persulfate and a reducible sulfur compound selected from the group consisting of thio-cyanates, sulfites and 60 thio-sulfates, said bath having a pH of about 1 to about 2.

9. A bath suitable for producing decorative, ornamental or utilitarian finishes on nickel articles and containing about 50 to about 200 grams 65 of ammonium persulfate per liter having an ammonium thio-cyanate concentration of about 0.5% and having a pH of about 1 to about 2.

10. A bath suitable for producing decorative, ornamental or utilitarian finishes on nickel articles and containing about 50 to about 200 grams of ammonium persulfate per liter and a small but effective amount of a reducible sulfur compound selected from the group consisting of thio-cyanates, sulfites and thio-sulfates. 70 75

11. A bath suitable for producing decorative, ornamental or utilitarian finishes on nickel articles and containing about 50 to about 200 grams of ammonium persulfate per liter, a small but effective amount of a soluble ferric salt and sufficient ammonium thio-cyanate to produce a red color in said bath.
12. A bath suitable for producing decorative, ornamental or utilitarian finishes on nickel articles and containing about 50 to about 200 grams of ammonium persulfate, about 25 to about 100 grams of sodium sulfate per liter, a small but effective amount to about 10 grams per liter of a soluble ferric salt and at least sufficient ammonium thio-cyanate to produce a red color in said bath.
13. A bath suitable for producing decorative, ornamental or utilitarian finishes on nickel articles and containing about 50 to about 200 grams of ammonium persulfate and about 1 to about 10 grams of ferric sulfate per liter and at least sufficient ammonium thio-cyanate to produce a red color therein.
14. A bath suitable for producing decorative, ornamental or utilitarian finishes on nickel articles and containing about 200 grams of ammonium persulfate, about 100 grams of sodium sulfate and about 10 grams of ferric sulfate per liter and at least sufficient ammonium thio-cyanate to produce a red color therein.
15. A bath suitable for producing decorative, ornamental or utilitarian finishes on nickel and nickel surfaced articles and containing an effective amount of hydrogen peroxide, a small but effective amount of a reducible sulfur-containing compound and sufficient of an acid selected from the group consisting of monochloracetic acid, orthophosphoric and sulfuric to produce a pH of about 1 to about 2.
16. A bath suitable for producing decorative, ornamental or utilitarian finishes on nickel and nickel surfaced articles and containing about 0.5 grams per liter of potassium thio-cyanate, about 5.0 grams per liter of sulfuric acid and about 25 cc. of 30% hydrogen peroxide per liter, said bath having a pH of about 1.2.
17. A bath suitable for producing decorative, ornamental or utilitarian finishes on nickel and nickel surfaced articles and containing an effective amount of a reducible sulfur compound, about 10 cc. to about 25 cc. of 30% hydrogen peroxide per liter and about 10 grams per liter of a buffer selected from the group consisting of monochloracetic acid and orthophosphoric acid.
18. A buffered bath suitable for producing decorative, ornamental or utilitarian finishes on nickel and nickel surfaced articles containing effective amounts of hydrogen peroxide and a sulfur compound reducible at the surface of said articles.
19. A buffered bath having a pH of about 1 to about 2 suitable for producing decorative, ornamental or utilitarian finishes on nickel and nickel surfaced articles containing effective amounts of hydrogen peroxide and a sulfur compound reducible at the surface of said articles.
20. As a new article of manufacture, a nickel body having a gray to black finish produced by simple immersion in a bath containing an oxidizing agent having a negative oxidation-reduction potential of at least -1.75 volts and a sulfur compound.
21. As a new article of manufacture, a nickel article having a series of colors produced by interference effect, said colors including those of the second order and being produced in a bath containing an oxidizing agent having an oxidation-reduction potential of at least -1.75 volts and a reducible sulfur compound.
22. A process for producing decorative, ornamental and utilitarian finishes on nickel surfaced articles which comprises subjecting nickel surfaced articles to the action of a bath having a pH of about 1 to about 2 and containing effective amounts of hydrogen peroxide and a sulfur containing compound reducible at said nickel surfaces at a temperature of about 15° C. to about the boiling point of the bath.
23. A process for producing decorative, ornamental and utilitarian finishes on nickel and nickel surfaced articles which comprises subjecting such articles to the action of a bath containing about 10 to about 25 cc. of 30% hydrogen peroxide per liter, about 10 grams per liter of an acid selected from the group consisting of monochloracetic acid, orthophosphoric acid and sulfuric acid and an effective amount to about 5 grams per liter of potassium thio-cyanate at a temperature of about 20° C.

BURTON BOWER KNAPP. 50